

## UNITED STATES PATENT OFFICE

2,411,113

## TREATMENT OF POLYENE COMPOUNDS

Anderson W. Ralston, Chicago, and Otto Turinsky, Palatine, Ill., assignors to Armour and Company, Chicago, Ill., a corporation of Illinois

No Drawing. Application January 22, 1942,  
Serial No. 427,834

6 Claims. (Cl. 260—405.6)

1

This invention relates to processes of treating polyene organic compounds and it more specifically relates to the treatment of unconjugated polyene organic material, such as fats and fatty acids having a plurality of double bonds with inorganic iodides of elements of the third, fourth and fifth groups of the periodic table of elements, whereby the unconjugated polyene materials are converted to conjugated polyene products or to products having improved drying or resinifying qualities.

It has hitherto been recognized that the chemical properties of unsaturated organic compounds having a plurality of double bonds depend not only upon the degree of unsaturation but also upon the relative position of the unsaturated bonds with respect to each other. If the unsaturated bonds are conjugated then the organic compound has properties characteristic of unsaturated compounds, and in addition, has those chemical properties characteristic of conjugated systems.

The distinction between conjugated and unconjugated systems is well illustrated by comparing the chemical behavior of linolenic acid and eleostearic acid. These acids are isomeric, straight chain fatty acids each containing three double bonds. It is believed that in linolenic acid the double bonds are in the 9—10, 12—13 and 15—16 position while in eleostearic acid they occupy the 9—10, 11—12 and 13—14 positions. Thus in eleostearic acid the double bonds are conjugated. When linseed oil is used as a paint vehicle the paint dries quite differently than it would if eleostearic acid were used. Eleostearic acid is the chief fatty acid constituent present in tung oil glycerides. Tung oil "body-dries" whereas linseed oil "film-dries." Body-drying is much preferred and is believed to result from the fact that eleostearic acid is conjugated.

Therefore, it is highly desirable that ways be developed by means of which unconjugated highly unsaturated compounds can be converted to conjugated, unsaturated compounds and thus gain the advantages inherent in conjugated systems.

The fact that the relative position of double bonds in an alkyl chain can be changed by treatment with strong alkalies has been known for some time. In Biochem. J. 31, 138 (1937) Moore reported that treatment of fats and fatty acids with alcoholic potassium hydroxide brings about a shift in the relative position of double bonds in an alkyl group and that this shift is towards a conjugated configuration. Recently Kass and Burr, J. Am. Chem. Soc. 61, 3292 (1939) have shown that the time necessary to bring about this

2

change can be materially reduced by the use of high boiling organic solvents and strong alkalies. Other investigators have found that the alkali process may be improved by conducting the reaction in aqueous solution at elevated temperatures and pressures. However, any such process which employs alkali has inherent disadvantages. In order to conduct this process it is necessary that the fats or fatty acids be converted to soaps. These soaps must then be acidified in order to obtain the transformed fatty acids. Where one desires to conjugate an oil a number of steps are, therefore, necessary in order to produce desired results by these processes. It is necessary to first saponify the fat and then to treat the soaps with strong caustic in order to bring about conjugation, acidify the resulting soaps, purify the fatty acids and finally reesterify them with glycerine.

It would be extremely desirable to develop a process whereby the unconjugated fatty acids or fats could be treated directly without the necessity of saponification or other chemical change. Such a process would be much easier to conduct on a commercial scale and would have a number of apparent advantages over the alkali processes for bringing about this transformation. Even before the introduction of the alkali methods various investigators have sought to find compounds which would produce the desired isomerization directly. For example, the Schrieber Patent No. 1,896,467 lists a number of compounds including sulfuric acid, ferrous iodide, chlorine, oxygen, etc., for this purpose; but none of these compounds have proved effective or have come into commercial use.

We have now discovered a class of compounds which catalytically improve to a very marked degree the drying or resinifying properties of unconjugated systems. This improvement involves a change of the unconjugated unsaturated system to a conjugated unsaturated system but we cannot definitely state that all the improvement in drying properties is explained by this transformation. The substances which we use to bring about this transformation are used in relatively small amounts at elevated temperatures which shows that they function as true catalysts. The class of compounds we use can be generally described as inorganic iodides of elements of the third, fourth and fifth groups of the periodic table of elements. Such iodides include iodides of phosphorus, tin, aluminum, antimony, and arsenic, these being representative elements of the third, fourth and fifth groups which form iodides. Iodides of aluminum have been found particularly desirable in our improved process.

In practicing our process the unconjugated

substance to be treated is admixed with small amounts of one or more of said iodides and then the mixture is heated to produce a shifting of the double bonds whereby a conjugated compound is formed. In general we can treat any organic polyene compounds which contains double bonds in unconjugated relation. Of the natural oils, linseed oil and soya bean oil are particularly susceptible to this treatment, and castor oil and fish oil are also markedly improved by the treatment. Other oils, such as cottonseed oil, peanut oil, corn oil and other oils not ordinarily regarded as drying oils, can also be treated by this procedure and their drying characteristics substantially improved. Instead of treating the oils directly, we can hydrolyze the oils to obtain the natural mixtures of fatty acids and then subject the mixture to the treatment for producing conjugation. The conjugated mixtures thus prepared may suitably be reacted with a polyhydric alcohol and a dibasic acid to form alkyd resins, or may be re-esterified with glycerol or the higher alcohols such as pentaerythritol or dipentaerythritol to form synthetic glycerides having improved drying characteristics.

Particularly in connection with the oils which are not normally classed as drying oils, such as cottonseed oil, corn oil, peanut oil, soyabean oil, etc., we find that especially good results can be obtained by first subjecting the acid mixture obtained from such an oil to fractional distillation and then subjecting a relatively low boiling volatile fraction so obtained and containing a higher proportion of the polyene acids, to the catalytic treatment described above.

Another procedure includes first subjecting the acids obtained through hydrolysis of natural oils to solvent extraction whereby there is produced a portion which contains unsaturated acids in greater proportion than in the original acid mixture, and then subjecting this portion to catalytic treatment as before described or, additional benefits may be obtained by first fractionally distilling the acid mixture, treating the fraction so obtained by solvent extraction, and then catalytically treating the resulting product using the herein disclosed inorganic iodides as the catalyst.

Though our improved process finds its greatest advantage in connection with those oils or natural mixtures of fatty acids which are classed as unconjugated oils or acids, the process can also be used to advantage in connection with oils and acids normally classed as conjugated but containing appreciable amounts of unconjugated compounds. Dehydrated castor oil is one of those products normally considered conjugated, but it does contain amounts of unconjugated compounds and it is markedly improved by the catalytic treatment described herein.

We shall now give examples of specific ways of practicing our process.

#### Example 1

Seven-hundred and fifty-seven parts by weight of linoleic acid which contains approximately 40% of oleic acid was weighed into a suitable reaction vessel. A stream of nitrogen gas was bubbled through the mixture both during the heating and cooling period, as presently described, to serve as a means of agitation and to supply an inert atmosphere. The mixture was heated to 255° C. and one part by weight of phosphorous iodide added. The temperature was held between 255° C. and 260° C. throughout the remainder of the heating period. Two more portions of 0.5

part by weight each of phosphorous iodide were added eight minutes and sixteen minutes, respectively, after the addition of the first portion. Heating was discontinued and the flask was cooled rapidly when the rate of increase in refractive index dropped off materially. Thus the total heating time in the presence of phosphorous iodide was twenty-five minutes. The refractive index of the original fatty acid mixture was  $n_{20}=1.4663$  which remained substantially constant until the phosphorous iodide was added. The refractive index after treatment was

$$n_{20}=1.4716$$

15 The iodine value dropped from 135 to 105 during treatment and the diene value increased from an initial value of 2 to a final value of 34.3. These values indicate that appreciable conjugation has been brought about by means of this treatment.

#### Example 2

Sixteen parts by weight of linoleic acid which contained approximately 35% of oleic acid and 0.016 part by weight of stannic iodide were mixed together. A stream of nitrogen gas was passed over the surface of the mixture both during the heating and cooling period. The test tube and its contents were heated in an air bath. After three minutes the temperature was 200° C. The heating was discontinued after 15 minutes, the temperature having attained a value of 345° C.

25 The refractive index of the original fatty acid mixture was  $n_{20}=1.4672$  and the refractive index after treatment was  $n_{20}=1.4738$ . The iodine value of the original fatty acid mixture was 144 which dropped to 117 after treatment. The diene value of the original mixture was 2 and attained a value of 24.3 as a result of the treatment. These values indicate that appreciable conjugation has 30 been brought about by means of this treatment.

#### Example 3

Three-hundred and thirty-nine parts by weight of refined soybean oil was weighed into a reaction vessel. The vessel was equipped with a motor stirrer to give efficient agitation. A stream of nitrogen gas was passed over the surface both during the heating and cooling period. The mixture was continuously stirred and heated to a temperature of 265° C. Phosphorous iodide was then added in approximately 0.1 part by weight quantities throughout the heating period. The 45 total heating time in the presence of the catalyst was 2 hours and 20 minutes. The temperature was allowed to increase gradually to 300° C. The total amount of phosphorous iodide added was 2.2 parts by weight. The refractive index of the original oil was  $n_{20}=1.4753$  which remained constant until the phosphorous iodide was added. The refractive index after treatment was  $n_{20}=1.4797$ . The iodine value dropped from 133 to 109 during treatment and the diene value increased from an initial value of 1.5 to a final value of 10.0. When spread on glass the above 50 treated oil dried giving a film which appeared "frosted," a characteristic of those oils in which there occur unsaturated conjugated systems. These data indicate that appreciable conjugation has been brought about by means of this treatment.

#### Example 4

Three-hundred and seventeen parts by weight of linoleic acid containing 30% of oleic acid was 55 heated to 260° C. with continuous stirring under

an atmosphere of nitrogen. When the temperature reached 260° C., 0.15 part by weight of aluminum triiodide was added and the reaction mixture was maintained at 260° C. for 35 minutes after which time 0.1 part by weight of aluminum triiodide was added and the mixture heated for seven minutes. Then an additional 0.01 part by weight of aluminum triiodide was added. The total heating time was 42 minutes, and the temperature ranged during this period from 260° C. to 270° C. The addition of the catalyst brought about a rapid rise in refractive index, and the heating was discontinued when the rate increase of refractive index was markedly lower. After 42 minutes, heating was discontinued and the fatty acids cooled rapidly.

The following data shows changes resulting from this treatment:

|                               | Before treatment | After treatment |
|-------------------------------|------------------|-----------------|
| Refractive index ( $n_{20}$ ) | 1.4668           | 1.4734          |
| Iodine value                  | 145              | 101             |
| Diene value                   | 1.5              | 26.6            |
| Action with stannic chloride  | Very slight      | Gelled.         |

These results indicate that appreciable conjugation has been brought about by this treatment.

#### Example 5

Three-hundred and seventeen parts by weight of the linoleic-oleic acid mixture described in the preceding example was heated to 260° C. with continuous stirring in an atmosphere of nitrogen. The catalyst in this case was antimony triiodide which was added in three portions, that is, 0.1 part by weight was added when the temperature attained 260° C., an additional 0.2 part by weight was added 20 minutes later, and a final 0.1 part by weight was added 50 minutes after the first addition. The reaction temperature varied from 260° C. to 270° C. The addition of the catalyst brought about rapid rise in refractive index, and the heating was discontinued when this rate of rise in refractive index was markedly lower. The total heating time in this case was 60 minutes, after which time the fatty acids were rapidly cooled in an atmosphere of nitrogen.

The following examination of the sample before treatment and after treatment show that appreciable conjugation has been brought about by this process.

|                               | Before treatment | After treatment |
|-------------------------------|------------------|-----------------|
| Refractive index ( $n_{20}$ ) | 1.4668           | 1.4729          |
| Iodine value                  | 145              | 117             |
| Diene value                   | 1.5              | 14.6            |
| Action with stannic chloride  | Slight           | Gelled.         |

#### Example 6

Three-hundred and two parts by weight of the linoleic-oleic acid mixture described in the preceding example was heated to 260° C. with continuous stirring under an atmosphere of nitrogen. When the temperature attained 260° C., 0.2 part by weight of arsenic triiodide was added and the heating continued for 35 minutes, after which time 0.03 part by weight of arsenic triiodide was added. The total heating time under these conditions was 40 minutes and the temperature varied from 260° C. to 270° C. The heating was discontinued when the rate of rise

of the refractive index was markedly lower. When the heating was discontinued, the fatty acids were rapidly cooled in an atmosphere of nitrogen. The following analytical data shows that appreciable conjugation has been brought about by this procedure.

|                               | Before treatment | After treatment |
|-------------------------------|------------------|-----------------|
| Refractive index ( $n_{20}$ ) | 1.4668           | 1.4733          |
| Iodine value                  | 145              | 108.2           |
| Diene value                   | 1.5              | 21.2            |
| Action with stannic chloride  | Slight           | Gelled.         |

#### Example 7

Fourteen-hundred parts by weight of extracted soy bean oil were treated with a catalyst which was prepared as follows: Eight parts by weight of iodine and 7 parts by weight of aluminum turnings were mixed with 30 parts by weight of carbon disulfide and the mixture refluxed for about 20 minutes. After this time the color of the iodine had completely disappeared indicating the formation of aluminum triiodide. Since an excess of aluminum was employed, the remainder was unreacted and was present as metallic aluminum. The catalytic mixture was then added to the soy bean oil and this mixture was then heated to 170° under an atmosphere of nitrogen and with sufficient stirring until the refractive index of the oil showed no further increase. This required a total time of 48 minutes. There was a marked increase in the refractive index of the oil at the time the temperature reached a value of 130° C. It required an additional 20 minutes heating time to raise the temperature to 170° C., and the mixture was then heated for an additional 20 minutes at this temperature. After this heating period, the reaction mixture was cooled under an atmosphere of nitrogen. The constants of the oil before and after treatment were as follows:

|                               | Before treatment      | After treatment                           |
|-------------------------------|-----------------------|-------------------------------------------|
| Refractive index ( $n_{20}$ ) | 1.4750                | 1.4836                                    |
| Iodine value                  | 134.4                 | 101.6                                     |
| Diene value                   | 1.5                   | 33.9                                      |
| Drying behavior               | Not dry in 200 hours. | Slightly tacky; frosted film in 18 hours. |
| Reaction of stannic chloride  | Non-gelling           | Immediate rubbery gel.                    |

These analytical constants and observations show that appreciable conjugation has been brought about in this soy bean oil by this treatment.

#### Example 8

The catalyst employed was aluminum triiodide which was prepared in a manner similar to that described under the previous example. The only difference in the catalyst used in this example and in the previous example was that 16 parts by weight of iodine were employed instead of 8 parts by weight as in the former example. The catalyst mixture was added to 1400 parts by weight of raw linseed oil and the heating was conducted as described in the foregoing example. The oil showed a marked increase in refractive index when the temperature reached 125° C. It required 52 minutes to heat the oil to 160° C. and the refractive index became constant 36 minutes later with the temperature rising slowly to 180° C. The reaction mixture was then cooled under an atmosphere of nitrogen

and the following analytical constants recorded:

|                               | Before treatment           | After treatment                              |   |
|-------------------------------|----------------------------|----------------------------------------------|---|
| Refractive index ( $n_{20}$ ) | 1.4810                     | 1.4916                                       | 5 |
| Iodine value                  | 177.8                      | 142.5                                        |   |
| Diene value                   | 1.8                        | 27.0                                         |   |
| Drying behavior               | Very tacky after 96 hours. | Slightly tacky; frosted film after 15 hours. |   |
| Reaction of stannic chloride. | Non-gelling                | Immediately rubbery gel.                     |   |

*Example 9*

The catalyst was prepared by shaking together 1.2 parts by weight of iodine, 1 part by weight of phosphorus and 10 parts by weight of carbon disulfide. This was added to 195 parts by weight of extracted soy bean oil and the mixture was heated in an atmosphere of nitrogen with sufficient stirring. At the end of 15 minutes the temperature rose to 150° at which time the refractive index of the oil showed appreciable increase. The temperature was permitted to rise slowly and after an additional 68 minutes, it had reached 178° C. at which time the refractive index showed no further increase. The reaction mixture was then cooled in an atmosphere of nitrogen. The following analytical constants and observations were obtained upon the initial and the starting materials.

|                                 | Before treatment      | After treatment        |    |
|---------------------------------|-----------------------|------------------------|----|
| Refractive index ( $n_{20}$ )   | 1.4750                | 1.4811                 | 35 |
| Iodine value                    | 134.4                 | 102                    |    |
| Diene value                     | 1.5                   | 18.0                   |    |
| Drying behavior                 | Not dry in 200 hours. | Dry after 70 hours.    |    |
| Reaction with stannic chloride. | Non-gelling           | Rubberly gel in 5 min. |    |

These analytical constants and observations show that the oil has been appreciably conjugated by this treatment.

In all instances the fatty acids which have been catalytically treated in the above described processes, can be esterified to form esters, and can be used in the arts wherever the use of conjugated unsaturated fatty acid esters is desirable.

In the foregoing examples wherein iodine and phosphorus or aluminum or other element of the third, fourth and fifth groups are brought together and the resulting product added to the oil or fatty acid, it is desirable to have a slight excess of the metal element present. However, as the foregoing examples show, an excess of the metal is not essential.

The oil or other polyene compound, after treatment in accordance with our process, need not be separated from the catalyst for most uses to which the treated oil is to be put. However, the catalyst can be separated from the treated material by the application of conventional caustic refining processes.

The amount of catalyst required is small. The amounts given in the foregoing examples have been found to give good results but still lesser quantities may be employed. More than the quantities stated can, of course, be used but this is wasteful and serves no useful purpose. If desired the catalyst may be removed from the final oil by any of the usual refining methods, but in general we prefer not to remove it since its presence is usually not harmful.

During the heating and cooling it is of special advantage to maintain the reaction mixture in an inert atmosphere such as nitrogen or carbon

dioxide, as we have found that this practice yields a product of a desired character having improved color and drying characteristics. However, our invention may be practiced without this feature.

We can operate at various times and temperatures. One of the characteristics of our invention is that conjugation is imparted quite rapidly, and this is a definite commercial advantage. Our oils and fatty acids can be heated for longer periods of time, if, for example, it is desired to impart bodied characteristics to the oil rather than conclude the heat treatment after conjugation alone has been imparted to the oil or fatty acid. That is to say, conjugated, unsaturated fatty acids and glycerides thicken when heated for somewhat longer periods of time than we have indicated in our examples. Therefore, we can, of course, impart conjugation to the unsaturated compound during a relatively short period and continue the heating for a longer period of time, up to two or three hours, if we wish to "body" the oil or fatty acid. Such thickened oils have much higher viscosity than the simple conjugated fluid oils, and this may be the result of polymerization of the conjugated material present. Therefore, we do not wish our invention to be limited to any particular time of heating. Those skilled in the art will understand different oils may require different heating periods and that the oil or fatty acid is to be heated until appreciable improvement in diene value is secured and that heat is to be discontinued before this product is bodied more than is desired.

Similar considerations apply with respect to temperature. At the temperature stated conjugation is imparted rapidly. Lower temperatures can be used but with a relatively slower reaction rate. For example, we can operate at temperatures below 100° C. and under certain conditions this has been found to be advantageous. Obviously, the temperature should not exceed the volatilization temperature of the material undergoing treatment, nor should it be so high as to decompose the oil or fatty acid. But within these operative limits suitable temperatures can be chosen.

Having thus described our invention, what we claim as new and desire to secure by Letters Patent is:

1. The process of conjugating a polyene compound chosen from the group consisting of unconjugated polyene fats and fatty acids which comprises heating said polyene compound in the presence of an inorganic iodide chosen from the group consisting of iodides of elements of the third, fourth and fifth groups of the periodic system, and discontinuing said heating after substantial conjugation of said polyene compound has been effected, but before the thus conjugated polyene compound becomes substantially heat bodied.
2. The process as in claim 1 wherein the iodide is phosphorous iodide.
3. The process as in claim 1 wherein the iodide is aluminum iodide.
4. The process as in claim 1 wherein the polyene compound is soy bean oil.
5. The process as in claim 1 wherein the polyene compound is linseed oil.
6. The process as in claim 1 wherein the polyene compound is heated at a temperature of about 200° C. to 300° C.

ANDERSON W. RALSTON.  
OTTO TURINSKY.